

April 26, 1932.

E. PUGH

1,855,869

METHOD OF AND APPARATUS FOR COATING ARTICLES

Filed Dec. 31, 1928

2 Sheets-Sheet 1



Inventor  
Emerson Pugh  
By *Malstrom Atty.*

April 26, 1932.

E. PUGH

1,855,869

METHOD OF AND APPARATUS FOR COATING ARTICLES

Filed Dec. 31, 1928

2 Sheets-Sheet 2



Fig. 3.



Fig. 4.

Inventor  
Emerson Pugh  
By *N. Patterson Atty.*

## UNITED STATES PATENT OFFICE

EMERSON PUGH, OF DOWNTON GROVE, ILLINOIS, ASSIGNOR TO WESTERN ELECTRIC COMPANY, INCORPORATED, OF NEW YORK, N. Y., A CORPORATION OF NEW YORK

## METHOD OF AND APPARATUS FOR COATING ARTICLES

Application filed December 31, 1928. Serial No. 329,593.

This invention relates to methods of and apparatus for coating articles, and more particularly to methods of and apparatus for finishing metal parts.

The principal objects of the invention are to provide a simple and expeditious method of and apparatus for applying material uniformly to exposed surfaces of articles.

In order to accomplish these objects in accordance with the invention, one embodiment thereof contemplates the conveying of metal parts or other articles to be coated through a closed chamber, the parts on the conveyor being connected in their passage therethrough to one terminal of a source of electrical energy of high potential. The opposite terminal of this source is connected to a nozzle through which an atomized spray of coating material is introduced into the chamber, thus giving the particles of the coating material suspended in the atmosphere of the chamber a charge opposite to that of the metal parts. These particles are thus selectively attracted to the uncoated portions of the parts in preference to the portions already covered by the solvent of the japan or other coating material so that they are deposited upon the uncoated surfaces thereof. To prevent the undue deposition of particles of coating material upon the interior of the chamber, the chamber wall is connected to the source of electrical energy so that it has the same potential as the nozzle.

It is believed that a complete understanding of the invention may be had from the following detailed description, taken in conjunction with the accompanying drawings, in which

Fig. 1 is a fragmentary plan view of an apparatus embodying features of the invention and which may be employed in practicing the method;

Fig. 2 is a front elevational view thereof with the front wall of the chamber removed;

Fig. 3 is an enlarged sectional view taken

on line 3—3 of Fig. 2, showing the electrical equipment associated with the apparatus, and

Fig. 4 is an enlarged perspective view of one of the supports for carrying the parts to be coated.

Referring now to the drawings wherein the same reference numerals indicate similar parts throughout the various views, the numeral 10 designates a chamber made of sheet metal having four pairs of swinging doors 55 11—11 which are so mounted as to always return to a closed position. This arrangement divides the chamber into three compartments 12, 13 and 14 so that compartments 12 and 14 serve as air locks for the middle compartment 13. Partitions 22—22 (Fig. 3) are provided under each pair of swinging doors 11—11 to prevent the circulation of air between the compartments. At both ends of the chamber 10 are sprockets 15—15 and 16—16 suitably mounted on shafts 17 and 18, respectively, and adapted to engage operatively and support an endless sprocket chain 20 in its passage through the chamber. Secured to the chain at equal spaces throughout its length are supports 25 for carrying parts 26 to be coated.

Each of the supports 25 includes an insulator 27 rigidly held in an upright position by a pair of angular members 28—28 secured to the sides of the chain 20. A metal cap 29 secured to the lower end of the insulator 27 is connected to a metal rod 30 mounted in the center of the insulator and terminating near the upper end thereof in a pair of laterally 80 extending arms 31—31 which are provided with hook portions 32—32 for supporting the parts 26 to be coated. At the upper end of the insulator 27 is a substantially rectangular guard 35 rigidly fastened thereto by a pin 85 36. This guard extends out beyond and surrounds the hook portions 32—32 so as to engage the swinging doors 11—11 and thus prevent injury to the parts 26 in their passage through the chamber.

5 A current conducting rail 40 for making contact with the metal caps 29 of the supports 25, is insulatively mounted on the bottom of the chamber 10 by means of insulating blocks 41-41 and is connected to the negative terminal 43 of a source of uni-directional electrical energy produced by a mechanical rectifier 44 (Fig. 3) from a source of alternating current (not shown). The positive 10 terminal 42 of the rectifier 44 is connected to the walls of the chamber 10 and also to a plurality of atomizing devices 45 suitably mounted alongside the chamber, as illustrated in Figs. 1 and 3.

15 Each of the atomizing devices 45 comprises a nozzle 50 connected to a source of compressed air (not shown) and having its forward end attached to the upper end of a tube 51, the lower end of the tube being immersed 20 in a liquified coating material 52, such as japan, lacquer, paint, etc., within a container 53. From the foregoing description it will be readily understood that upon compressed air being admitted to the nozzle 50, the emission 25 of the air past the upper end of the tube 51 creates a vacuum therein whereby the liquified coating material 52 is drawn up in the tube and the force of the air breaks the coating material into finely divided particles and 30 blows it into the middle compartment 13 through apertures 55 in a wall of the chamber 10.

In practicing the invention, the shaft 17 is 35 connected to and driven by any suitable source of power (not shown) so as to rotate the sprockets 15-15 keyed thereto and effect the movement of the sprocket chain 20 in the direction indicated by the arrows in Figs. 1 and 2. With the negative terminal 43 of 40 the mechanical rectifier 44 connected to the current conducting rail 40 by a conductor 59, and the positive terminal 42 connected to the chamber 10 and the nozzle 50 by a conductor 60, the mechanical rectifier is operated to 45 create a uni-directional current of high potential. The parts 26 to be coated are then placed on the hook portions 32-32 of the metal rods 30, and as the guards 35 engage and open the doors 11-11 in passing from 50 compartment 12 into compartment 13 of the chamber 10, the metal caps 29 make contact with the current conducting rail 40. This contact connects the parts 26 to the negative 55 terminal of the source of uni-directional electrical energy through laterally extending arms 31-31, metal rod and cap 30, 29, respectively, contact rail 40, and conductor 59 to the negative terminal 43 of the mechanical rectifier 44. As has been previously explained, the nozzle 50 of the atomizing device 45 is connected to a source of compressed air to effect the introduction of a coating material 52 in finely divided particles into the compartment 13. Since the atomizing device is 60 connected to the positive terminal of the 65

source of uni-directional electrical energy through nozzle 50, conductor 60 to the positive terminal 42 of the mechanical rectifier 44, the particles of coating material are given a positive charge as they emerge from the 70 atomizing device 45 into the compartment 13 through apertures 55 in the chamber 10. The negatively charged parts 26 to be coated attract the positively charged particles of coating material so that the latter is deposited 75 upon the surface of the parts 26 to form coatings thereon. A uniform coating of each part is assured, due to the fact that as the particles of the coating material are deposited thereon, the solvent of the coating material acts as 80 a dielectric, whereby the positive charge is intensified at the uncoated spots on the parts 26 to better attract the particles of coating material thereto.

The difference of electrical potential 85 between the parts 26 to be coated and the atomizing devices 45 can be varied greatly, depending on size of the chamber, the characteristics of the particular coating material used and the speed imparted to the conveying 90 chain 20, but the voltage should not be of such a value as to cause arcs between the parts being coated and the atomizing devices or chamber walls. The connecting of the walls 95 of the chamber 10 and the atomizing devices 45 to the same terminal of the source of uni-directional electrical energy produces positive charges on both the coating material 52 and the walls of the chamber 10 so that the 100 particles of coating material are repelled from the walls to prevent undue deposition thereon. In order to carry off any excess coating material, the bottom of the chamber 10 is sloped toward a drain 64 (Fig. 3).

As the finished parts emerge from the 105 chamber 10, they are removed from the supports 25 and uncoated parts are placed on the hook portions 32-32 and they in turn are carried through the chamber 10 so that the 110 process is a continuous one.

It will be understood that the embodiment 115 of the invention herein described and illustrated is merely a convenient and useful form of the invention which is capable of many other modifications without departing from the spirit and scope of the invention.

What is claimed is:

1. A method of applying a finish to an article of manufacture, consisting in finely dividing a coating material, surrounding the 120 article of manufacture to be coated with an atmosphere having the finely divided material suspended therein, and subjecting the article of manufacture and the particles of the material to a difference of electrical potential to cause the material to be attracted to and deposited upon the article of manufacture.

2. A method of applying a finish to an article of manufacture, consisting in producing a 130 uni-directional current of high voltage in an

atmosphere, introducing a coating material in a finely divided form into the atmosphere, and subjecting the article of manufacture to be coated to the current and the atmosphere for a predetermined period of time to cause electrical deposition of the material upon the article of manufacture.

3. A method of applying a finish to an article of manufacture, consisting in enclosing an article of manufacture to be coated, connecting a supply of coating material and the article of manufacture to be coated to opposite terminals of a source of uni-directional current of high voltage, introducing an atomized coating material into the enclosed atmosphere, and subjecting the enclosure to the same potential as the coating material to repel the particles of coating material therefrom as they are attracted and deposited upon the article of manufacture.

4. In an apparatus for applying a finish to an article of manufacture, a chamber for enclosing the article of manufacture to be coated, an air lock therefor, means for introducing into the chamber coating material in finely divided form, means for conveying the article of manufacture through the air lock into the chamber, means for connecting the article of manufacture for a predetermined period of time to one terminal of a source of uni-directional energy, and means for connecting the coating material to the opposite terminal of the source of electrical energy to cause the deposition of the coating material upon the article of manufacture.

5. In an apparatus for applying a finish to an article of manufacture, a closed chamber for receiving an article of manufacture to be coated, an atomizing device for introducing a spray of coating material into the chamber and a source of electrical energy associated with the chamber for subjecting the article of manufacture to one potential and the atomizing device and the chamber to an opposite potential to cause the deposition of the coating material upon the article of manufacture and prevent the deposition thereof upon the chamber wall.

6. In an apparatus for applying a finish to an article of manufacture, a chamber for enclosing the articles of manufacture to be coated, means for conveying the articles of manufacture therethrough at predetermined intervals, means for connecting the articles of manufacture to one terminal of a source of electrical energy at a predetermined time, an atomizing device for injecting particles of a coating material into the chamber, and means for connecting the atomizing device and the walls of the chamber to the opposite terminal of the source of electrical energy to repel the particles of coating material from the walls as they are attracted to and deposited upon the articles of manufacture.

7. A method of applying a finish to an arti-

cle of manufacture consisting in enclosing a space of predetermined size, introducing into the enclosed atmosphere a coating material in a finely divided form, conveying the articles of manufacture to be coated through the enclosed atmosphere in spaced relation, and subjecting the articles of manufacture and the coating material to a difference of electrical potential to cause the coating material to be deposited on the articles of manufacture.

8. A method of supplying a finish to an article of manufacture consisting in enclosing an article of manufacture to be coated, connecting a supply of coating material and the article of manufacture to be coated to opposite terminals of a source of uni-directional current of high voltage, introducing an atomized coating material into the enclosed atmosphere, subjecting the enclosure to the same potential as the coating material to repel the particles of coating material therefrom as they are attracted and deposited upon the articles of manufacture, and imparting movement to the article of manufacture relative to the enclosure.

9. In an apparatus for applying a finish to an article of manufacture, a chamber for enclosing the articles of manufacture to be coated, a conveyor for moving the articles of manufacture therethrough at predetermined intervals, means carried by the conveyor for electrically connecting the articles of manufacture to one terminal of a source of electrical energy at a predetermined time, an atomizing device for injecting particles of a coating material into the chamber, and means for connecting the atomizing device and the walls of the chamber to the opposite terminal of the source of electrical energy to repel the particles of coating material from the walls as they are attracted to and deposited upon the articles of manufacture.

10. In an apparatus for applying a finish to an article of manufacture, a chamber for enclosing the articles of manufacture to be coated, a conveyor for moving the articles of manufacture therethrough at predetermined intervals, means carried by the conveyor for carrying the articles of manufacture, means for cooperating with said carrying means for electrically connecting the articles of manufacture to one terminal of a source of electrical energy at a predetermined time, an atomizing device for injecting particles of the coating material into the chamber, and means for connecting the atomizing device and the walls of the chamber to the opposite terminal of the source of electrical energy to repel the particles of coating material from the walls as they are attracted to and deposited upon the articles of manufacture.

11. A method of applying a finish to an article of manufacture, consisting in enclosing a space of predetermined size, introduc-

ing into the enclosed atmosphere a coating material in a finely divided form, conveying the article of manufacture to be coated through the enclosed atmosphere, and subjecting the article of manufacture and the coating material to a difference of electrical potential to cause the coating material to be deposited on the article of manufacture.

In witness whereof, I hereunto subscribe my name this 19th day of December, A. D. 1928.

EMERSON PUGH.

#### DISCLAIMER

1,855,869.—*Emerson Pugh*, Downers Grove, Ill. METHOD OF AND APPARATUS FOR COATING ARTICLES. Patent dated April 26, 1932. Disclaimer filed November 10, 1936, by the patentee; the assignee, *Western Electric Company, Inc.*, assenting and concurring.

Hereby enters this disclaimer to claims 2 and 11 in said specification.  
[*Official Gazette December 8, 1936.*]

25

30

35

40

45

50

55

65

ing into the enclosed atmosphere a coating material in a finely divided form, conveying the article of manufacture to be coated through the enclosed atmosphere, and subjecting the article of manufacture and the coating material to a difference of electrical potential to cause the coating material to be deposited on the article of manufacture.

In witness whereof, I hereunto subscribe my name this 19th day of December, A. D. 1928.

EMERSON PUGH.

#### DISCLAIMER

1,855,869.—*Emerson Pugh*, Downers Grove, Ill. METHOD OF AND APPARATUS FOR COATING ARTICLES. Patent dated April 26, 1932. Disclaimer filed November 10, 1936, by the patentee; the assignee, *Western Electric Company, Inc.*, assenting and concurring.

Hereby enters this disclaimer to claims 2 and 11 in said specification.  
[*Official Gazette December 8, 1936.*]

25

30

35

40

45

50

55

65

## DISCLAIMER

1,855,869.—*Emerson Pugh*, Downers Grove, Ill. METHOD OF AND APPARATUS FOR COATING ARTICLES. Patent dated April 26, 1932. Disclaimer filed November 10, 1936, by the patentee; the assignee, *Western Electric Company, Inc.*, assenting and concurring.

Hereby enters this disclaimer to claims 2 and 11 in said specification.  
[*Official Gazette December 8, 1936.*]